

July 8, 1947.

C. D. ENDER

2,423,555

COATED PAPER PRODUCT

Filed April 24, 1944



CLARENCE D. ENDER  
INVENTOR.

BY *Ernest G. Peterson*

AGENT

## UNITED STATES PATENT OFFICE

2,423,555

## COATED PAPER PRODUCT

Clarence D. Ender, Wilmington, Del., assignor to  
Hercules Powder Company, Wilmington, Del.,  
a corporation of Delaware

Application April 24, 1944, Serial No. 532,463

2 Claims. (CL. 117—111)

1

This invention relates to coating compositions and more particularly to the application of coating compositions to porous fibrous materials to obtain extremely thin but impervious coatings.

When employed on porous materials, coating solutions tend to impregnate the material. At least one sizing treatment has usually been found necessary before the coating solution could be applied. A sizing operation by filling pores of the material acts to retard impregnation and resultant waste of the more valuable coating solution. But an uneven surface is nevertheless presented to the first application of coating solution. Consequently, some tiny, porous particles usually project through the film coating, breaking its continuity. The coating solution applied in succeeding coats is then drawn by capillary action through these particles into the material. Tiny, imperceptible pinholes may persist in this manner even though several coats are applied. The weight of coating required to build up over the projecting particles and seal the pinholes has been found so great as to be uneconomical and makes the coated material unsuited for some purposes. Thus, thin and impervious coatings on porous materials have been difficult to prepare.

Now in accordance with this invention, a relatively thick mass or coat of a solution of chlorinated rubber having a nonvolatile content and viscosity within certain limits, whereby impregnation is avoided, is applied to a web of porous paper. The web then is drawn across a doctor while applying pressure to the web where in contact with the doctor, whereby the doctor by its wiping and spreading action draws out the coating solution to a thin continuous film. The volatile solvent is permitted to evaporate. As a result of its high nonvolatile content, the thin film remains continuous and substantially non-flowing during drying. By utilizing a coating composition containing between about 40% and about 80% chlorinated rubber, between about 15% and about 50% plasticizer, for example, dissolved in a volatile solvent to form a solution containing between about 40% and about 80% nonvolatile materials and having a viscosity between about 600 and about 600,000 cp., in the particular coating procedure set forth, there is obtained a coating which is thinner than about 0.0010 in. or is lighter in weight than about 15 lbs. per ream of 3600 sq. ft. This film is impervious to moisture, oil, grease, nitrated glycerol, nitrated glycols, and the like.

Having now indicated in a general way the nature and purpose of the invention, there follows a more detailed description of a preferred embodiment thereof with reference to the accompanying drawing.

The figure represents a diagrammatic side ele-

2

vation view of a knife coater suitable for carrying out the process of the invention.

Referring to the drawing, the paper to be coated 1 is fed from a reel 2 over tension rolls 3 and 4 and then is picked up by a flexible blanket or belt 5 which provides the motive force for the paper. The blanket or belt is resilient and may be of rubber. The tension rolls are so adjusted that the paper is held firmly upon the blanket.

The speed of the blanket is governed by power-driven rolls 6. In general, the speed of the blanket is held between about 15 and about 30 ft. per minute.

15 The coating composition 7 is poured, for example, upon the paper using an adjustable funnel 8 and allowed to spread roughly over it as the paper approaches a doctor knife 9. The knife may be raised or lowered. It is adjusted so that it exerts pressure upon the paper, which, supported upon the resilient blanket, is held firmly against the knife at all times. The knife wipes and spreads the composition and removes excess composition. In its action it draws the coating to a very thin, uniform continuous film. The knife is supported by a strong backing 10 which may contain a heating element. Thus, the knife may be heated so as to coat solutions too viscous at room temperature.

20 30 The doctor utilized to spread the initially coated film and to draw it to a very thin film is preferably a rigid doctor knife or blade, preferably with a rounded edge. However, any doctor capable of drawing the highly viscous solution coated to a very thin film, for example, a reverse roll doctor, rod doctor, or the like, forced against the coating web, may be used.

It is preferred that the paper or like web be

40 45 50 55 60 pressed firmly by or against the doctor edge or surface. As shown by the drawing, a convenient method for applying pressure to the paper against a rigid doctor involves support of the paper by a resilient supporting means, such as a resilient rubber blanket which may be, for example, between about 0.25 and about 2 inches thick. Such a blanket supports the paper web, preventing breakage, and at the same time strongly presses it against the doctor. It also serves by frictional engagement to pull the paper past the doctor. Accordingly, a preferred embodiment of the present invention involves coating a web, engaging the coated web with a rigid doctor, resiliently supporting and pressing the web against the doctor, and drawing the web while so pressed across the working surface or edge of the doctor to draw and thin out the coating. Other means of exerting pressure against the doctor, as by a hard or resilient roll opposite the doctor, may be em-

ployed.

The coated material 11 then passes to a dryer or other means for dissipating the solvent.

An alternative procedure involves applying the coating composition to the web by means of a roll-type applicator. The lower part of the applicator dips in a container of the coating solution. The paper or like web is pressed firmly against the applicator's upper surface. A scraping knife applied to the applicator roll may act as a regulator of the quantity of coating composition permitted to pass to the paper. The paper, coated with the desired amount of composition, is drawn across a doctor roll or knife which wipes and spreads the composition. Preferably, the doctor is adjusted so that it exerts pressure upon the paper in order to draw the coating to as thin a uniform, continuous film as possible, but this is not essential.

In Table I are given a number of particular formulas as examples of coating compositions used in the process according to this invention. Chlorinated rubber and plasticizer are essential ingredients; resins, waxes, fillers, and the like are optional; compositions comprising chlorinated rubber, a plasticizer, a wax, and a resin are preferred.

The ingredients are dissolved in a volatile inert solvent to form a solution which, at the temperature of coating, has a viscosity between about 600 and about 600,000 cp., preferably between 2,000 and 100,000 cp. It is essential that the viscosity be in this range to avoid impregnation of the material and to permit the film to be drawn out thinly to provide imperviousness in one coat. The nonvolatile content of the solution will be between about 40% and about 80% by weight of the solution, preferably between 50% and 70%. The ranges given are critical. Too low a nonvolatile content gives a coating which may contain pinholes due to shrinkage and flow of the drawn film before drying; too high a nonvolatile content makes a very thin coating too difficult to obtain as it prevents proper drawing-out; i. e., workability, of the composition.

The composition for convenience is preferably applied at temperatures between about 20° C. and about 35° C., that is, at ordinary room temperatures. More viscous solutions may be applied at elevated temperatures, up to about 80° C. Temperatures above about 80° C. must be avoided as too rapid evaporation of solvent occurs during the coating, adversely affecting the uniformity and continuity of the coating and increasing the possibility of pinholes. The viscosity of solutions may sometimes be increased by cooling to below room temperature, if desired, say to about 0° C.

It has been found that to form a coating substantially impervious to moisture and most oils and liquids, a minimum weight of about 4 lbs. of coating per ream of 3600 sq. ft. is required, when coated on one side of the paper, about 2 lbs. per ream of 3600 sq. ft. when applied to both sides of the paper. The minimum weight of coating is preferred. Such a film has a thickness of about 0.0001 inch. The maximum weight of coating will be governed by economy, by the type of paper used, and by other requirements. For example, where the coated paper is to be used for dynamite wrappers, a weight of coating above about 30 lbs. per ream of 3600 sq. ft. coated on one side of the paper is undesirable since on exploding the dynamite in closed places, as in mines, excessive quantities of poisonous or irritating gases are formed. Such a film has a thickness of about 0.0008 inch.

In general, a weight of coating between about 4 and about 18 lbs. per ream of 3600 sq. ft. is most satisfactory.

The chlorinated rubber used in this invention must have a chlorine content between about 60% and about 75%, preferably between 60% and 69%. Its viscosity characteristic should be between about 20 and about 1,000 cp. The viscosity of the composition solution is directly related to the viscosity of the chlorinated rubber; the chlorinated rubber should have a viscosity within the limits given to obtain a final solution within the critical viscosity range.

Plasticizers that have been found satisfactory include dibutyl phthalate, diamyl phthalate, butyl acetyl ricinoleate, butyl stearate, tricresyl phosphate, triethyl citrate, triphenyl phosphate, dibutyl tartrate, linseed oil, castor oil, soybean oil, tung oil, etc. A plasticizer is essential to retention of imperviousness after coating. It is used in a quantity between about 15% and about 50% by weight of the nonvolatile ingredients.

Waxes which may be used in the composition include paraffin, beeswax, tallow, japan, carnauba, candelilla, montan, spermaceti, white ceresin, palm, or any waxy substance, such as stearic acid, vaseline, cetyl palmitate, oxidized paraffin, octadecyl palmitate, oleyl hydroxyoleate, oleyl oleate, cetyl oleate, ceryl cerotate, myricyl 30 palmitate, myricyl cerotate, etc. Waxes impart moisture-vapor-proofness. They may be used in a quantity up to about 5% by weight of the nonvolatile ingredients of the composition.

Resins that have been employed include rosin; 35 rosin maleates; ester gum; hydrogenated rosin; hydrogenated methyl abietate; ethylene glycol ester of rosin or hydrogenated rosin; pentaerythritol ester of rosin; diethylene, tetraethylene, or hexaethylene ester of hydrogenated rosin; polymerized rosin; natural resins; alkyd resins; phenol-formaldehyde resins; urea-formaldehyde resins; coumarone-indene resins; terpene resins; etc. Resins may be incorporated in a quantity up to about 25% of the nonvolatile ingredients.

The composition essentially contains a suitable solvent or solvent mixture which will effectively dissolve the chlorinated rubber, plasticizer, and other ingredients where included, and which may be dissipated following application of the composition to the material being coated. The solvent acts merely as a vehicle for the application of the composition. Such a solvent may be a hydrocarbon, such as xylene, toluene, benzene, mesitylene, ethyl benzene, high aromatic content petroleum naphtha, cyclohexane, high-flash naphtha, etc.; an ester, such as hexyl acetate, butyl acetate, methyl acetate, etc.; a ketone, such as methyl-ethyl ketone, methyl isobutyl ketone, etc.

The proportions of the nonvolatile ingredients in the composition will in general be as follows: Chlorinated rubber, between about 40% and about 80%, preferably between 55% and 75%. Plasticizer, between about 15% and about 50%, preferably between 20% and 36%. Wax, between about 0% and about 5%, preferably between 2% and 4%. Resin, between about 0% and about 25%, preferably between 10% and 20%.

The presence of water in the composition solution is undesirable and should be avoided, the adherence and smoothness of the coating being adversely affected. Pinholes tend to form where the water droplets were.

The method according to this invention may be used to coat various porous, fibrous materials. In particular, it is useful for coating papers, such as wrapping, bond, ledger, text, and kraft paper, etc., and fibrous sheets, such as jute, cardboard, Bristol board, fiber board, Lion jute tag cardboard, etc.

Paper coated with this composition may be made into dynamite cartridges and packed with dynamite in the usual manner. Such wrappers, made impervious to nitroglycerin and moisture by a coating of extreme thinness, have in consequence better explosive properties and improved oxygen balance.

tion is 40-80% by weight and the viscosity of the composition is 600 to 600,000 centipoises by the falling ball method at the temperature of application used, and drawing out the composition by pressure of a doctor against the moving paper while resiliently supported, to a continuous coating which, when dry, will have a thickness from about 0.0001 to about 0.0008 inch and a weight no greater than 30 pounds per ream of 3600 square feet, and drying the resulting coating.

2. A method for applying to paper extremely thin coatings of chlorinated rubber, impervious to moisture and most oils, which comprises applying to a moving, continuous web of the paper a viscous composition comprising chlorinated rubber in a quantity between 40% and 80%, plasticizer between 15% and 50%, 0-5% wax, 0-25% resin, the percentages being by weight of total nonvolatile components of the composition, and volatile solvent for the chlorinated rubber and other ingredients, the solvent being in a quantity such that the nonvolatile content of the composition is 40-80% by weight and the viscosity of the composition is 600 to 600,000 centipoises by the falling ball method at the temperature of application used, supporting the moving paper web on a resilient belt or blanket, passing the paper against

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10

10&lt;/div

**Certificate of Correction**

Patent No. 2,423,555.

July 8, 1947.

**CLARENCE D. ENDER**

It is hereby certified that error appears in the printed specification of the above numbered patent requiring correction as follows: Column 6, line 37, claim 2, for "60-70%" read 60-75%; and that the said Letters Patent should be read with this correction therein that the same may conform to the record of the case in the Patent Office.

Signed and sealed this 2nd day of September, A. D. 1947.

[~~SEAL~~]

**LESLIE FRAZER,**  
*First Assistant Commissioner of Patents.*